

## UNITED STATES PATENT OFFICE

2,514,330

## MIXED BASE LUBRICATING GREASES

Arnold J. Morway, Clark Township, Union County, and Rosemary O'Halloran, Elizabeth, N. J., assignors to Standard Oil Development Company, a corporation of Delaware

No Drawing. Application June 5, 1948,  
Serial No. 31,398

4 Claims. (Cl. 252—40)

1

The present invention relates to mixed base lubricating greases and particularly to soda-barium soap greases which are particularly suited for the lubrication of high speed anti-friction bearings over a broad temperature range. The invention relates further to a process for producing greases of the type referred to and to the improvement of viscosity-temperature characteristics of such greases.

In U. S. Patent No. 2,245,702 to Morway, one of the present inventors, there is described a mixed base grease prepared from the mixed soaps of soda and baryta which has been found fairly satisfactory for the lubrication of anti-friction bearings. The composition described in said patent, however, has certain deficiencies in that it is not useful over as wide a temperature range as may be desired and its viscosity and consistency vary considerably with wide changes in temperature. The grease described in said patent contains a slight excess of alkali, for example from 0.05 to 0.3%. The composition described therein becomes fibrous at temperatures of about 230° to 240° F.

It has now been found that unexpected improvements in mixed soda-barium grease may be obtained by employing fatty acids of average lower molecular weight than the acids used in the prior art and by employment of a base lubricating oil of high viscosity index. In addition, it has been found that if the finished grease contains a small amount of free acid rather than free alkali as in the aforesaid patent, a change in physical structure of the grease is permitted at high temperatures which makes the lubricant suitable for anti-friction bearings running at high speeds and at elevated temperatures.

It is well known that most lubricating greases pass through a change of phase at a temperature in the approximate vicinity of the melting point of the fat or fatty acid from which the thickening soap is prepared. The phase change occurring at this point, i. e. the uni-dimensional melting point of the soap, is slight. However, at higher temperatures another phase change occurs which is due to increased thermal energy in the soap lattice and is called the bi-dimensional melting point. By the latter expression is meant the phenomenon by which a soap structure which exists in three dimensions breaks down in the

2

second of such dimensions. At such a phase change or transition point, lubricating greases lose their short fibered smooth structure and become very fibrous and rubbery in character.

If the change in phase referred to above occurs in a lubricating grease below the desired operating temperature, the grease is not a good lubricant. Since anti-friction bearings under many operating conditions attain temperatures considerably higher than the normal transition or phase change temperature of greases, it is desirable to change the transition temperature. The present invention is based upon the discovery that this can be accomplished by using a fatty acid of shorter chain length, or lower molecular weight, in producing the grease-forming soap. Apparently such a reduction in the molecular weight or chain length also decreases the solvency of the soap in the mineral oil. In addition, by the use of more aliphatic type mineral oils, i. e. paraffinic or predominantly paraffinic as distinguished from naphthenic or aromatic, the soap solvency in the oil is further decreased. This further raises the temperature at which phase change or transition takes place. These results can be obtained without so far reducing solvency of the mineral oil for the soaps that the soaps will separate from the oil on cooling.

The use of a high viscosity index oil, that is an oil that is more paraffinic than customarily used in grease manufacture, not only raises the transition temperature but also gives a product which has better temperature-viscosity relationship. The latter is an obvious advantage of the use of oil of high viscosity index but the former is quite unexpected and is contrary to the general custom of using low viscosity index oils for most lubricating greases. As a result, lubricants prepared according to the present invention may be used at extremely low temperatures as well as at very high temperatures, comparatively speaking.

By employing the three factors mentioned above, namely, the shorter average length of the fatty acid chain, a base lubricating oil of high viscosity index, and a slight excess of acidity as distinguished from the prior art excess of alkalinity, several improvements may be obtained. Because of the lower solvency of the soaps, greases of a desired consistency or hardness may

be obtained with relatively less soap. Thus the soap content may be as low as 3 or 4% although it may also go as high as 25 or 30% by weight, based on the finished grease, if a very stiff lubricant is desired. These greases obviously have more body at higher temperatures and less at lower temperatures because of the high viscosity index oil used and they give outstanding performance on the high temperature-high speed spindle test. Such greases have excellent shear stability and do not break down upon severe mechanical working.

#### EXAMPLE

As one example of a grease made according to the present invention, the following formula was employed:

12.50% hydrogenated fish oil fatty acids (predominately palmitic acid)  
 1.70% sodium hydroxide  
 0.78% barium hydroxide octahydrate  
 0.40% phenyl-alpha naphthylamine antioxidant  
 71.87% extracted Panhandle distillate (150 vis./100, SUS)  
 12.80% extracted Coastal distillate (80 vis./100, SUS)

The fatty acids which comprised about 57% palmitic and 16% myristic, with small amounts of higher acids, were mixed with part of the lubricating oil and heated to a temperature of about 150° F. The barium hydroxide, in the form of a 10% hot aqueous solution was added and the temperature was maintained therein until the baryta was entirely taken up by the fatty acids. The sodium hydroxide was next added, also as an aqueous solution, and the temperature was increased to 240° F. and maintained until all water was evaporated. Thereafter the soap concentrate was heated further as the remainder of the lubricating oil was added slowly. This was continued until the soap was completely dispersed in the mineral oil at a temperature of between 375° and 425° F. The grease was then poured into pans for cooling and homogenized to the desired consistency at room temperatures.

Although the foregoing is a desirable method for preparing greases of the mixed soda-barium type, they can easily be prepared by other well known methods. The temperatures employed may be as low as 350° or as high as 500° F. or more if desired. Hydrogenated fish oil acids which have an average composition of less than 18 carbon atoms per molecule and more than 14 are very satisfactory but other acids may be used if desired. In general, the fatty acids having 14 to 18 carbon atoms and even slightly higher acids in minor proportions are quite suitable, but it is important that the average should be at least slightly less than the composition of stearic acid, i. e. 18 carbon atoms. Otherwise, oil solubility of the soaps is too great to realize the full benefits of this invention. Similarly, if the average composition is C<sub>14</sub> or lower, the oil insolubility is too great. Simple acids such as lauric, myristic, or palmitic may be used in mixtures with each other or with stearic acid as desired to obtain the proper average.

The grease in the example, as noted above, was prepared from a base oil composed predominantly of extracted Panhandle distillate with a small amount of extracted Coastal distillate. The viscosity index of the combined oils was about 93.

For comparative purposes, two similar compositions were prepared from other oils and sub-

jected to high speed spindle tests at a temperature of 250° F. The first was prepared from a straight Coastal distillate having a viscosity index of 50 and the second from a Rodessa distillate having a viscosity index of 113. The performance data are shown in Table 1.

TABLE 1

|    | Mineral Oil                          | Performance of Soda-Barium Greases at 250° F. |                    |
|----|--------------------------------------|-----------------------------------------------|--------------------|
|    |                                      | Coastal Distillate                            | Rodessa Distillate |
| 15 | Vis./210° F., SUS.....               | 42                                            | 44                 |
|    | Viscosity Index.....                 | 50                                            | 113                |
|    | Hrs. Spindle Life at 10,000 RPM..... | 100-300                                       | 500-1100           |

The spindle test apparatus used in these runs is the ABEC-NLGI Committee Test as described in the Committee's Technical Bulletin No. 5. It consists of a 204 type ball bearing mounted on a belt-driven spindle under a thrust load of 14-15 p. s. i. This is operated at 250° F. and 10,000 R. P. M. on a 22-hour cycle, (2 hours at room temperature) until failure occurs. Failure occurs when the bearing is running under such friction that the operating temperature rises 25° F., thus activating a shut-off system.

Although oil of high viscosity index appears to be most desirable as the basic lubricant in these greases, it is found Panhandle mineral oil distillates show exceptionally good high temperature performance characteristics which is not to be expected even from their viscosity index. The Rodessa type distillates have substantially higher viscosity index, but as indicated in Table 2, the Panhandle product with a viscosity index of 100 showed an even better high speed spindle life.

TABLE 2

|    | Mineral Oil                          | Performance of Soda-Barium Greases at 250° F. |                    |
|----|--------------------------------------|-----------------------------------------------|--------------------|
|    |                                      | Panhandle Distillate                          | Rodessa Distillate |
| 45 | Vis./210° F., SUS.....               | 44                                            | 44                 |
|    | Viscosity Index.....                 | 100                                           | 113                |
|    | Hrs. Spindle Life at 10,000 RPM..... | 1,874                                         | 500-1,100          |

In general, the low temperature properties of a grease are governed by its soap content, and the pour point and viscosity (at the test temperature) of its mineral oil. Therefore, improvements in performance may be obtained by lowering any of these factors. Dewaxing, or dilution of the mineral oil, or lowering the soap content are all possibilities.

Dewaxing the Panhandle distillate from its original +30° F. pour point to 0° F. pour point definitely improves its low temperature characteristics at -40° F., 17.4 sec./rev., as compared to 37.1 sec./rev. However, this grease did not have as good high temperature characteristics as the undewaxed stock as shown in Table 3.

TABLE 3

|    |                                                  | Solvent 150 Neutral (Undewaxed) | Solvent 150 Neutral (Dewaxed) |
|----|--------------------------------------------------|---------------------------------|-------------------------------|
|    |                                                  |                                 |                               |
| 70 | Mineral Oil, ASTM Pour Point, °F.....            | +30                             | 0                             |
|    | Low Temperature Torque, Sec./Rev. at -40° F..... | 37.1                            | 17.4                          |
|    | Hours Spindle Life at 10,000 RPM and 250° F..... | 1,874                           | 623                           |

The qualities of this Panhandle stock are of such a nature that the base oil can be diluted with an extracted Coastal distillate in order to improve the low temperature properties of the grease, without materially affecting the high temperature performance. Such a composition was used in Example 1. In this way a grease of an excellent combination of properties can be produced.

The comparative properties of a straight Panhandle distillate and of a Panhandle distillate mixed with 15% of Coastal distillate, as in the Example 1, are shown in Table 4. It will be noted particularly that the low temperature torque is substantially lower in the mixed oil lubricant than in the straight Panhandle distillate grease. This suggests that where low temperature operation is contemplated, the Coastal distillate may be used in minor proportions at only a slight sacrifice of high temperature spindle life.

TABLE 4

## Performance of soda-barium greases

| Type Mineral Oil                                                | Panhandle Distillate | Panhandle Distillate + Coastal Distillate |      |
|-----------------------------------------------------------------|----------------------|-------------------------------------------|------|
| Vis. S. S. U. at 210° F.                                        | 44                   | 44                                        | 42.5 |
| V. I.                                                           | 100                  | 100                                       | 93   |
| Per Cent Soap Content                                           | 15.6                 | 12.5                                      | 15.6 |
| Spindle life, hrs.                                              | 1,874                |                                           | 1657 |
| Low temp. torque test, sec./rev. at 40° F., 2000 gm. cm. torque | 37.1                 | 23.9                                      | 8.5  |

<sup>1</sup> Soap prepared from commercial hydrogenated fish oil acids containing 35.2% C<sub>18</sub>, 28% C<sub>16</sub>, 15% C<sub>20</sub> acids.

For normal anti-friction bearing greases, a soap content of 20 to 25% or more, is frequently used. Because of the high yield value of the mixed soda-barium greases of this invention, products of approximately the same consistency may be produced with only about 13 or 14% of soap, where suitable fatty acids of shorter average chain lengths are used to form the soaps. This is of advantage because a large soap content adversely affects the low temperature performance of the grease as indicated by a torque of 37.1 for a grease containing 15.6% soap as compared with torque of 23.9 for the same type of grease containing 12.5% soap, Table 4.

The use of a minimum soap content is advantageous for reasons of economy as well as for improved low temperature performance. By using soaps prepared from acids of shorter average chain length than stearic acid (C<sub>18</sub>) greases of a given consistency may be obtained with decreased soap content, due to the relatively lower oil solubility of the soaps of lower acids. The oil thickening effect of a given quantity of soap increases as oil solubility decreases. Where higher fatty acids are used more soap is required to give the grease a stable structure. Also, such soaps increase the torque resistance of the grease at low temperature, as shown in Table 4.

Hydrogenated fish oil acids of different types vary in composition as regards the chain length of their constituents. Thus one commercial fatty acid marketed as "51-HO" contained 15.8% myristic (C<sub>14</sub>) acid, 56.6% palmitic (C<sub>16</sub>) acid, 20.4% stearic (C<sub>18</sub>) acid, 3.4% arachidic (C<sub>20</sub>) acid and 1.3% behenic (C<sub>22</sub>) acid. Another, sold under the trade name "Hydrofol 51" contained 8.5% myristic, 35.2% palmitic, 28.2% stearic and 15.0% and 8.8%, respectively, of arachidic and behenic acids. The former was used in the ex-

ample, above, whereas the latter was used in the greases of Table 4.

Greases prepared with soaps of higher fatty acid, i. e. acids of longer average chain length, show greater torque, when used in the same oil, but the difference in oils employed is also of some importance, as indicated below in Table 5. It should be noted that greases containing as little as 12.5% soap, as in Table 4, second column, are too soft for use at elevated temperatures because of poor shear stability. The grease of Table 5 contained about 15% soda-barium soaps of "Hydrofol 51" acids.

TABLE 5

|                                                        | Mineral Oil | Treated Coastal Distillate | Extracted Rodessa Distillate |
|--------------------------------------------------------|-------------|----------------------------|------------------------------|
| Vis. S. S. U. at 210° F.                               |             | 42                         | 44                           |
| V. I.                                                  | 50          |                            | 113                          |
| Torque test, sec./rev. at -40° F., 2000 gm. cm. torque | 47.3        |                            | 4.2                          |

It will be noted that the respective mineral oils of Table 5 had approximately the same viscosity at 210° F., but the Rodessa distillate had a much higher viscosity index.

Although the greases of this invention can be prepared with small amounts of excess free alkalinity as well as free acidity, it has been found that the presence of a small amount of free fatty acid substantially improves the high temperature performance of the product, without detriment to the oxidation resistance or shear stability. Evidently the free fatty acid has some solvency effect preventing the grease from becoming rubbery at the high test temperature. The data in Table 6 show the superior life of various greases containing about 16.5% by weight of soaps of "Hydrofol 51" acids, being acid and alkaline, respectively.

TABLE 6

## High temperature performance of soda-barium greases

| Free Reaction of Grease                                 | High Speed Spindle Life, Hours at 250° F. |                   |                           |                         |
|---------------------------------------------------------|-------------------------------------------|-------------------|---------------------------|-------------------------|
|                                                         | Treated Coastal                           | Extracted Coastal | Extracted Panhandle Dist. | Extracted Rodessa Dist. |
| Acid (about 0.3% by wt., calculated as free oleic acid) | 312                                       | 700               | 1,874                     | 1,058                   |
| Alkaline (about 0.1% by wt., calculated as free NaOH)   | 277                                       | 465               | 748                       | 775                     |

From the foregoing it will be seen that mixed base greases having excellent properties of shear stability, resistance to oxidation, yield values, and high temperature structure stability may be produced from the sodium-barium soaps of relatively low molecular weight fatty acids. As suggested above, the extracted Panhandle distillates are particularly desirable as base lubricating oils, but the invention is not limited to the use of such oils. In some cases, it is desirable to add some Coastal stock to cut back the extracted Panhandle because of the high pour point of the Panhandle. A mixture or blend having approximately the following characteristics appears to be highly suitable:

ble as a base for the greases of this invention, but the invention is not by any means limited thereto.

|                   |         |
|-------------------|---------|
| Vis./100° F., SUS | 143.1   |
| Vis./210° F., SUS | 42.5    |
| Vis. index        | 92      |
| Flash             | °F. 385 |
| Pour              | °F. +25 |

In general a lubricating grease prepared from oils of fairly high viscosity index, for example 80 to 125, thickened with 5 or 6 to 25 or 30%, preferably 10 to 20% of the mixed soda-barium soaps of hydrogenated fish oil acids or analogous products having an average of less than 18 carbon atoms and more than 14 carbon atoms, are quite suitable.

The proportions of barium soap to sodium soap may be varied rather widely as described in the Morway Patent 2,245,702.

The limitations stated therein are a sodium-barium soap weight ratio of from 1 to 1, to about 10 to 1 which corresponds to mol ratios of from about 1.2 to 1 to about 12 to 1. The limits in the case of the present type of compositions are greater, especially with regard to the upper limit, the overall range being between about 1 to 1 and 30 to 1, on a sodium soap/barium soap mol ratio basis. Preferably the mol ratio is in the range from about 15 to 1 to about 25 to 1. The preferred range in the present compositions is therefore considerably higher than the upper limit of the prior art compositions, which differ however in several other ways. Especially suitable is a mol ratio from about 17 to 1 to about 19 to 1.

The excess quantity of acid may be varied somewhat but should be kept rather low. In general it should be from as low as 0.01% and in general from 0.05 to 0.5% by weight calculated as free oleic acid.

It will be understood that the greases prepared according to this invention may contain conventional additives such as antioxidants, tackiness agents, extreme pressure additives, corrosion inhibitors, and other materials such as are well known in the art. It is generally preferred to include a small amount of a suitable antioxidant such as phenyl alpha naphthylamine or phenyl beta naphthylamine and the like, although such materials are not always required. When included they should be added in proportions of 0.1 to about 1% by weight, based on the composition, 0.4 or 0.5% usually being preferred. In general, the oil composition, which may include these additives and is referred to generally as "lubricating oil" in the claims should have V. I. of at least 80 and preferably 85 to 115. The oil will preferably comprise 75 to 94% of the composition and the soap from about 6 to 25%, although these limits may be exceeded for specific purposes.

What is claimed is:

1. An anti-friction bearing lubricating grease

consisting essentially of a mineral base lubricating oil having a viscosity index of at least 80 thickened to a grease consistency with a mixed sodium-barium soap of fatty acid having an average of less than 18 carbon atoms, wherein the molar ratio of soda soap to barium soap is between 1 to 1 and 30 to 1 said grease containing a slight excess of said fatty acid sufficient to give a free acidity of 0.01 to 0.5% by weight, calculated as free oleic acid.

2. A lubricating grease composition consisting essentially of 75 to 94% mineral base lubricating oil having a viscosity of 50 to 500 SSU at 100° F. and a viscosity index of between 85 and 115, and 6 to 25% of a mixed sodium-barium soap of hydrogenated fish oil acids having an average molecular composition of less than 18 carbon atoms and at least 14 atoms, wherein the molar ratio of soda soap to barium soap is between 1 to 1 and 30 to 1 said grease having a sufficient excess of said acids to give a free acidity of 0.05 to 0.5% by weight, calculated as oleic acid.

3. A lubricating grease consisting essentially of 80 to 90% mineral base lubricating oil having a viscosity index of at least 80, about 10 to 20% of mixed sodium-barium soaps of aliphatic carboxylic acids having an average composition of more than 14 and less than 18 carbon atoms, wherein the molar ratio of soda soap to barium soap is between 1 to 1 and 30 to 1 about 0.1 to 1% of an antioxidant, said grease having a sufficient excess of said acids to give a free acidity of about 0.01 to 0.5% by weight, calculated as free oleic acid.

4. A lubricating grease composition consisting essentially of a mineral base lubricating oil having a viscosity index between 80 and 125, and 5 to 30% of the mixed soda-barium soaps of hydrogenated fish oil acids having an average chain length between 14 and 18 carbon atoms, said soda soap exceeding said barium soap in molar proportions by at least 15 to 1, and said grease having a slight excess of said acids sufficient to give to said grease a free acidity of 0.01 to 0.5%, calculated as free oleic acid.

ARNOLD J. MORWAY,  
ROSEMARY O'HALLORAN,

#### REFERENCES CITED

50. The following references are of record in the file of this patent:

#### UNITED STATES PATENTS

| Number       | Name          | Date           |
|--------------|---------------|----------------|
| 55 2,005,553 | Miller        | June 18, 1935  |
| 2,245,702    | Morway        | June 17, 1941  |
| 2,318,847    | Flint et al.  | May 11, 1943   |
| 2,449,312    | Murray et al. | Sept. 14, 1948 |
| 2,451,039    | Morway et al. | Oct. 12, 1948  |
| 60 2,468,099 | Morway        | Apr. 26, 1949  |
| 2,487,080    | Swenson       | Nov. 8, 1949   |